

## UNITED STATES PATENT OFFICE

TORRENCE A. SWARTZ AND WILMER P. UHLER, OF TOTTENVILLE, NEW YORK

## ELECTRIC RESISTANCE MATERIAL

No Drawing.

Application filed September 24, 1923. Serial No. 664,575.

Our invention relates particularly to a composition of matter which may be formed to provide electrical resistance devices having extremely high resistive qualities.

It is well-known that in certain electrical devices, such as are employed in wireless apparatus and other highly sensitive instruments, it is necessary to employ resistance of extremely high value, and that resistance materials, as heretofore produced, lack the desired tensile and transverse strength and therefore have their limitations for installation. Furthermore, in resistance devices employing carbon and graphite coated surfaces, it is difficult to either secure or maintain uniformity and permanence of resistance value.

The principal objects of our invention are to provide an electrical resistance material that will not only afford the infinitely high resistive qualities required, but that will have the tensile and transverse strength desired, and that will maintain its uniformity and permanence.

Other objects of our invention are to provide an electric resistance material in which the electrical conducting medium may be so varied as to afford an extremely wide range of conductivity and that may be readily moulded or otherwise formed into any desired shape or drawn into wire if desired, and which may be flexed and connected in any desired manner.

The form of our invention as hereinafter described comprehends an electric resistance material formed of a composition of matter comprising rubber, sulphur and an inert substance serving as a filler, and finely divided particles of electrical conducting material uniformly embodied therein.

Our invention also includes all of the various novel features of production and embodiment as hereinafter more definitely specified.

We have found that a resistance material having extremely high electrical resistive qualities, combined with the desired features

of utility, may be produced by the composition comprising crude rubber, sulphur and an inert substance such as "blanc fixe" or "barium sulphate" ( $BaSo_4$ ) having embodied therein carbon, preferably in the form of lamp-black, gas-black, powdered graphite or other suitable finely divided electrical conducting materials, and that these combined substances may be conveniently mixed by the use of rubber mixing rollers in a well-known manner.

We have also found that desirable results may be attained by forming the composition of forty (40%) per cent rubber, twenty (20%) per cent sulphur, fifteen (15%) per cent-thirty-five (35%) per cent lamp-black, and twenty-five (25%) per cent-five (5%) per cent "blanc fixe". It is to be understood, however, that the proportions herein set forth may be widely varied to adapt the resulting resistance material to varying conditions that may be encountered.

The composition thus described may be conveniently moulded into suitable form and vulcanized, preferably to form vulcanite, and may be prepared for use in a variety of forms, such as plates, discs, bars, rods or wire that may be conveniently adapted to any conditions ordinarily found in commercial devices.

Our invention is advantageous in that it provides a non-fragile resistance material having an infinitely high resistance value, and consequently can be adapted to conditions not heretofore possible.

We do not desire to limit our invention to the specific materials and their proportions herein set forth, as it is obvious that various modifications may be made therein without departing from the spirit and scope of the invention as defined in the appended claims.

Having thus described our invention, we claim:—

1. An electrical resistance material comprising a vulcanized composition consisting

of rubber, sulphur, barium sulfate and finely divided particles of carbon, the relative proportions of said barium sulfate and carbon determining the specific resistivity of the material.

5 2. An electrical resistance material comprising a coherent vulcanized composition of approximately 40% of rubber, 20% of sulphur, 15 to 35% of lamp black, and 25 to 10 5% of barium sulfate.

10 In witness whereof, we have hereunto set our hands the 20th day of September, A. D., 1923, and the 20th day of September, A. D., 1923 respectively.

15 TORRENCE A. SWARTZ.  
WILMER P. UHLER.

20

25

30

35

40

45

50

55

60

65